

## UNITED STATES PATENT OFFICE

GEORGE A. RICHTER, OF BERLIN, NEW HAMPSHIRE, ASSIGNOR TO BROWN COMPANY, OF BERLIN, NEW HAMPSHIRE, A CORPORATION OF MAINE

## PROCESS OF ALKALINE FIBER LIBERATION

No Drawing.

Application filed February 28, 1930. Serial No. 432,272.

This invention relates to the production from raw cellulosic material, such as wood, of cellulosic pulps, by a two-step process of alkaline fiber liberation in which the alkaline liquors employed in both steps to dissolve the cementitious content of the raw cellulosic material consist of alkaline solutions similar in chemicals used to those employed in the so-called soda and kraft processes.

In the so-called soda and kraft processes of fiber liberation, the raw cellulosic material is cooked in comparatively dilute alkaline liquors under conditions of high temperature and pressure until fiber isolation has been accomplished. By neither the soda process, wherein a solution of caustic soda serves as the cooking liquor, nor by the kraft process, wherein a solution of both caustic soda and sodium sulphide serves as the cooking liquor, is it possible to produce pulps of low pentosan content, as dilute alkaline liquors, especially kraft liquors, are comparatively poor solvents for pentosans, even at elevated temperatures.

The object of the present invention is to make possible an economical utilization of the usual fiber liberating alkalies, such as employed in the soda or kraft processes, for the production of cellulose pulps having a much lower pentosan content than that of the usual soda or kraft pulps and excelling the usual soda or kraft pulps in other important respects, such as in softness, easy bleachability, and suitability for conversion into cellulose derivatives. In accordance with the process of the present invention, raw cellulosic material, such as chipped wood, is steeped for a considerable period of time in an alkaline liquor of high alkalinity but at a temperature little, if any, above that of the prevailing atmosphere. The free liquor is then separated from the cellulosic material and the cellulosic material is cooked to complete fiber liberation in a comparatively dilute alkaline liquor, which may include residual alkali associated with such material, a suitable amount of water, and added alkali. Such a two-step process has many features of advantage over the

usual one-step processes of alkali fiber liberation. Thus, I have found that liquors of high alkalinity extract substantial amounts of lignin, pentosans, less resistant celluloses, and resinous material from the raw wood at comparatively low temperatures, and, further, that the extraction of pentosans is favored by the low temperature. Hence the subsequent cooking of the wood to complete fiber liberation may be carried out in liquors of much lower alkalinity than that of the usual alkaline cooking liquors, as the partially extracted wood lends itself to much easier pulping than raw wood. The resulting product is of an alpha cellulose content significantly higher than that of the usual commercial wood pulps, such as sulphite, soda, or kraft, and after bleaching is far more valuable as a raw material for papermaking and in the preparation of cellulose derivatives. An important feature of a process such as described is that it may be carried out in a single alkaline digester, the concentrated liquor employed for the initial treatment being drained from the cellulosic material after the treatment, and the requisite amount of water containing alkali, if desired, then being added to the cellulosic material to produce a suitable dilute alkaline liquor in which cooking to complete fiber liberation may be effected. If desired, however, the initial treatment may be carried out in open tanks, whereupon after this treatment has been completed and the free alkaline liquor separated from the cellulosic material, the cellulosic material associated with residual alkali may be charged into alkaline digesters wherein fiber liberation is completed at high temperature and under pressure.

The initial treatment is carried out in a liquor containing from 10% to 25% alkali in the form of caustic soda or both caustic soda and sodium sulphide. The liquor may be maintained at room temperature or at somewhat higher temperatures, say, 50° C., particularly when sodium sulphide is present therein, as this chemical is more active upon lignin than is caustic soda, especially at temperatures somewhat higher than room temperature. At room temperature or below, a

liquor containing only caustic soda is especially active upon pentosans, so that when such a liquor is employed, a suitable oxidant may be added thereto to accelerate the removal of lignin at such temperature,—the permanganate, hypochlorite, or peroxide of sodium being especially suitable for this purpose. When wood is used as the raw cellulosic material, it is preferable to reduce it to chips of a size much smaller than those prepared for the usual chemical cooking processes. Thus, whereas the usual chip size ranges from  $\frac{1}{2}$ -inch to 1-inch in length, it is preferable to use chips of about  $\frac{1}{4}$ " length in the process of the present invention, as such chips make possible the shortening of the time required for the initial treatment and subsequent cooking. The time of the initial treatment may be from six to twenty-four hours, depending upon other factors, such as the strength and temperature of the liquor, the conditions under which subsequent cooking is to be effected, and the characteristics of the final product to be attained. Under a given set of factors, however, the time required for the initial treatment may be shortened by using small size chips or by accelerating the impregnation of the chips by confining them and forcing the treating liquor thereinto under the pressure of hydraulic pumps. When the product need not have papermaking characteristics, as, for example, when intended for the preparation of cellulose derivatives, the liquor may contain more than 25% caustic soda equivalent, but liquors of such strength are undesirable from the standpoint that, aside from injuring the fiber for papermaking, they react upon the cellulose itself and materially lower the yield of product.

When the initial treatment has been completed, the liquor is yellow or light brown in color and the chips have a corresponding color and are slippery to the touch. The liquor is drained from the mass of chips and after suitable fortification with alkali may be reused for the treatment of a fresh batch of chips, as the alkali consumption in a single use is relatively small. The alkali-soaked chips may then be washed, if necessary, until they have a residual alkali content sufficient, when diluted with the appropriate amount of water, to form a dilute alkaline liquor such as is necessary for cooking to complete fiber liberation. If, however, it is desired to produce pulp which may be bleached with ease in a single step to a white product of high alpha cellulose content, it is preferable to wash the alkali-soaked chips as free as possible from associated alkali, and then to treat the washed chips with chlorine water, which serves to remove ligneous and coloring matter or to convert this matter into reaction products readily soluble in the dilute alkaline liquor in which subsequent cooking is effected. Because a large proportion of the encrustations of the

wood has been removed by the initial treatment, the wood is considerably more porous than in its raw state and is accordingly penetrated much more rapidly and uniformly by the chlorine water than would be the case were the raw wood treated. The thoroughly washed chips may be steeped at room temperature in chlorine water containing from 4% to 6% chlorine, based on wood, for about four to six hours. Should there be traces of caustic soda in the wood, the chlorine water reacts therewith to produce sodium hypochlorite, the action of which upon ligneous and coloring matter is similar to that of chlorine.

When the washed chips are associated with sufficient alkali to permit carrying out the subsequent cooking operation, cooking is effected under the desired temperature conditions in a liquor made up of the residual alkali and water. If, however, the alkali-soaked chips have been thoroughly washed and then treated with chlorine water as hereinbefore described, they are again thoroughly washed after the chlorine water treatment and before cooking to complete fiber liberation in dilute alkaline liquor. The presence of sodium sulphide in the cooking liquor enhances the bleachability and strength of the pulp, so that when the initial treatment is carried out with a solution of caustic soda alone, and no subsequent treatment of the chips with chlorine water is effected, the mass of treated chips is preferably washed to a point where sodium sulphide may be added along with water thereto to produce a liquor of the desired low alkalinity and at the same time have the desired sodium sulphide content. When, however, the initial treatment is effected in a solution of both caustic soda and sodium sulphide in which the sodium sulphide is present in such proportion as is desired for subsequent cooking, the alkali-soaked chips resulting from the initial treatment may be washed to a point where the addition of water only thereto results in a cooking liquor of the desired alkalinity and sulphidity. In any case, however, cooking to complete fiber liberation is effected in a liquor of much lower alkalinity than that of the liquors employed in the production of soda or kraft pulp, for instance, in a liquor of an alkalinity about one-half that of the usual liquor employed in the production of kraft pulp.

A typical procedure falling within the purview of the present invention may be carried out substantially as follows. Wood chips, e. g., spruce, of about  $\frac{1}{4}$  to  $\frac{1}{2}$ -inch length, are steeped in a caustic soda solution of 18% strength at 20° C. for twelve hours, at the end of which time the chips and the solution have a decided yellow color, even though very little caustic soda has been consumed by reaction upon the encrustations of the wood. The chips are then drained free of

excess solution and are washed until they contain only about 25% to 35% caustic soda, based on wood. The chips are then transferred to an alkaline digester, if not already there, and sufficient water is added to cover the mass. The digester is closed and the charge therein is heated to a temperature of about 335° F., at which temperature the charge is maintained for three hours to complete fiber liberation. The yield of pulp obtained amounts to about 45% to 50%, based on wood, being hence comparable to the yields obtained in the usual processes of fiber liberation. The pulp, however, is materially higher in alpha cellulose content, which component amounts to about 93% to 95%. It has a strength and tear resistance approximating that of a usual, unbleached kraft pulp, but its pentosan content is much lower, amounting to only about 3% to 4%, as against the 8% to 10% pentosan content of the usual kraft pulp. Such a product may be used as such for papermaking, but when a white product is desired, it may be bleached with a hypochlorite liquor, as usual. When a white product is desired without decrease in alpha cellulose content, the unbleached pulp is preferably subjected to chemical refining prior to the bleaching operation. Such refining may include the treatment of the unbleached pulp with chlorine water containing, say, 3% to 5% chlorine, based on the weight of pulp at room temperature, for about two hours, at the end of which time the chlorine is practically consumed by reaction upon lignin and other coloring matter present in the pulp. The pulp is then washed free of chlorine water and soluble reaction products, whereupon it is digested in a dilute solution of a suitable alkali, for example, in a solution containing 5% to 10% caustic soda, based on pulp, at 210° to 212° for about four to five hours. The solution reacts upon and dissolves insoluble chlorinated coloring matter and other non-alpha cellulose components present in the pulp, so that the resulting product when washed free of alkaline liquor requires a hypochlorite liquor containing only 3% to 4% bleach, based on pulp, to become converted into a pure white product. Preferably, the bleach liquor contains, say, 1/4% to 1/2% caustic soda, which is sufficient to maintain a condition of distinct alkalinity throughout the bleaching operation, which condition militates against the formation of oxycelluloses or other undesirable reaction products. The bleached product has an alpha cellulose content of about 95%, or even higher, and is thus more refined than the raw or unbleached pulp resulting from the two-step process of fiber liberation. It is suitable for use as a cotton fiber substitute, both in the manufacture of high grade papers and in the preparation of cellulose derivatives.

When the finished pulp is intended pri-

marily as a papermaking raw material, it is preferable that cooking to complete fiber liberation be effected in a liquor containing sodium sulphide, as this chemical enhances the papermaking characteristics, i. e., the strength and tear resistance of the pulp. To this end, the alkali-soaked chips from the initial treatment may be washed until, say, only 10% to 15% caustic soda remains therein, whereupon cooking to complete fiber liberation may be effected in a liquor made up not only of the residual caustic soda associated with the chips, but also with about 10% to 15% sodium sulphide, based on wood. The raw pulp resulting from cooking in such a liquor has papermaking characteristics comparable to those of the best grade kraft pulp. It may be used as such, bleached, or refined and then bleached, as already described.

In addition to those advantages hereinbefore enumerated, the process of the present invention requires the utilization of comparatively little heat in producing a product characterized by its high content of alpha cellulose. Thus, the initial treatment takes place with the application of little, if any, heat, and the subsequent cooking to complete fiber liberation is accomplished in a period of time notably shorter than that of the usual chemical pulping processes. The process of the present invention may be expediently and economically practised in those mills where soda or kraft pulps are being produced, with little, if any, change in equipment or raw materials, as the regenerated or white liquors available in such mills are precisely the liquors required in the process. Moreover, the spent liquors produced in the practice of the present process may be mixed with the spent liquors produced in the soda or kraft mills, and the sodium constituent of the mixed liquors recovered in one recovery apparatus.

I am aware of the fact that it has been proposed to impregnate wood chips or other raw cellulosic material with the alkali necessary for cooking to complete fiber liberation by soaking in liquors of suitable strength and then cooking the alkali-impregnated wood in water. It has not heretofore been recognized, however, that alkaline liquors of above 10% caustic soda strength are especially effective in extracting undesirable components, especially pentosans, from wood chips, at about room temperature, and that if the chips are permitted to remain in contact with excess liquor of such strength for a sufficient period of time, subsequent cooking to complete fiber liberation may be effected in a liquor of about half the alkali content of the usual alkaline cooking liquors, to produce a pulp characterized by its high alpha cellulose content, its low pentosan content, and its excellence as a raw material.

both for papermaking and for conversion into cellulose derivatives.

I claim:

1. A process which comprises steeping raw cellulosic material at not greater than about room temperature in an alkaline liquor of a strength in excess of 10% caustic soda equivalent until a large proportion of the encrustations of such material has been dissolved, and then cooking the material at elevated temperature and under pressure in an alkaline liquor of much lower strength to complete fiber liberation.

15 2. A process which comprises steeping chipped wood at not greater than about room temperature in an alkaline liquor of a strength of about 10% to 25% caustic soda equivalent until the liquor has extracted sufficient encrusting material from the wood 20 to have a decided coloration, draining the free liquor from the wood, washing the wood until it contains only about 25% alkali based on wood, and cooking the wood to complete fiber liberation in an alkaline liquor formed by the addition of only water to such wood.

25 3. A process which comprises steeping chipped wood at not greater than about room temperature in an alkaline liquor of a strength in excess of 10% caustic soda equivalent for over six hours, and then cooking the wood at elevated temperature and under pressure to complete fiber liberation in an alkaline cooking liquor containing only about 25% caustic soda equivalent, based on wood.

30 4. A process which comprises steeping chipped wood at about room temperature in an alkaline liquor of a strength in excess of 10% caustic soda equivalent for over six hours, and then cooking the wood at elevated temperature and under pressure to complete fiber liberation in an alkaline cooking liquor containing sodium sulphide.

35 5. A process which comprises steeping chipped wood at about room temperature in an alkaline liquor of high alkalinity until a large proportion of the encrustations of such wood has been dissolved, washing, treating with chlorine water to react upon ligneous and other coloring matter in the wood, again 40 washing, and cooking in an alkaline liquor of low alkalinity to complete fiber liberation.

45 6. A process which comprises steeping chipped wood in a caustic soda solution of mercerizing strength at not greater than about room temperature until considerable of the pentosan content of such wood has been removed and such wood has become impregnated with solution, and cooking such 50 impregnated chips in an alkaline liquor of much lower strength to effect fiber libera- tion.

55 7. A process which comprises steeping chipped wood in a caustic soda solution of mercerizing strength at not greater than

about room temperature until considerable of the pentosan content of such wood has been removed and such wood has become impregnated with solution, and cooking such impregnated chips in only added water to effect fiber liberation.

In testimony whereof I have affixed my signature.

GEORGE A. RICHTER.

75

80

85

90

95

100

105

110

115

120

125

130